

## UNITED STATES PATENT OFFICE

2,636,850

ELECTROPLATING OF COPPER FROM  
CYANIDE ELECTROLYTES

George W. Jernstedt and James D. Patrick, Pittsburgh, Pa., assignors to Westinghouse Electric Corporation, East Pittsburgh, Pa., a corporation of Pennsylvania

No Drawing. Application February 18, 1949,  
Serial No. 77,265

3 Claims. (Cl. 204—52)

1

This invention relates to the electrodeposition of copper by means of periodic reverse current from cyanide electroplating electrolytes containing certain joint addition agents.

In Patent 2,451,341, there is disclosed the process of electroplating copper from an electrolyte containing copper in solution by employing a periodic reverse electric current. Specifically, a member to be plated with copper is immersed in the electroplating electrolyte and subjected to a flow of electrical current such that for a period of time of not over 40 seconds a plating electric current deposits copper on the member, and then for a shorter period of time a deplating electric current of such a magnitude is applied to the member that it delivers at least 10% of the coulombs of electric current delivered in the preceding plating period whereby a part of the plated copper is removed thereby leaving an increment composed of sound, smooth and relatively-uniform copper plate. Repetition of the alternate plating and deplating builds up the copper until a desired thickness of copper has been applied to the member. The copper plate so produced on the member is sounder, harder, smoother and more homogeneous than copper applied by previously-known processes. Numerous other unexpected advantages have been realized over any previously-known method of electroplating.

Specifically, periodic reverse current enables the electroplating of copper to be so carried out that one or more of the following advantages over continuous direct-current plating are obtained.

- (1) Increase in the rate of plating,
- (2) Increase in the density of the metal deposited,
- (3) Improved brightness of electrodeposited metal surface,
- (4) Greater smoothness in the electrodeposited metal,
- (5) Heavier deposits are platable,
- (6) Decreased porosity, and
- (7) Improved electrodeposited metal distribution on base members.

The periodic reverse current process may be so carried out that any one feature of the above seven can be emphasized. While this gives the electroplater a control of the plating process that was not available when employing only continuous direct current, or other conventional plating current cycles disclosed in the prior art, there are

2

instances where it is desirable to emphasize two or more of the above features at the same time. In particular, it is desirable to plate at the highest possible rate of copper deposition while producing a smooth, bright deposit. Obviously, there is a limit to the current density at which plating may be carried out while maintaining the resulting electrodeposit of metal smooth and bright, regardless of the mode of plating.

These are suggestions in the prior art that copper may be electrodeposited by direct current from a copper cyanide electrolyte while dissolved zinc is present in the electrolyte; see the article by Walter R. Meyer and Arthur Phillips on pages 400 and 401 of the Transactions of the Electrochemical Society, vol. LXXIII (1938). However, this article indicates that the sole benefit from zinc additions in copper electrolytes is a slight increase in brightness for very thin electro-deposits not thicker than one-half mil (0.0005 inch), while any thicker deposits become inferior having a distinct columnar structure with rougher surfaces than that of electroplated deposits of equal thickness obtained from the same copper electrolyte with no zinc present. The use of thiocyanate addition agents alone to copper cyanide electroplating electrolytes has been suggested previously for direct-current electroplating. Thiocyanate has been employed in direct-current electroplating with moderate benefits; however, other addition agents give superior results, and thiocyanates are not used to any great extent as an addition agent for copper cyanide electrolytes.

In accordance with this invention, it has been discovered that the electrodeposition of copper from aqueous cyanide electrolytes containing copper by periodic reverse current may be greatly improved by having present simultaneously in the electrolyte zinc and thiocyanate (CNS<sup>-</sup>). When operated with periodic reverse current, the presence of both zinc and the thiocyanate in particular proportions in copper cyanide electrolytes produces results markedly superior than with either alone.

The object of this invention is to provide for the electrodeposition of copper from aqueous copper cyanide electrolytes containing zinc and thiocyanate jointly in predetermined amounts, by means of a periodic reverse electric current.

A further object of this invention is to provide a process for the electrodeposition of smoother and brighter deposits of copper from cyanide electrolytes by maintaining predetermined amounts of both zinc and thiocyanate in

the electrolyte and passing a periodic reverse current through the electrolyte.

A still further object of the invention is to provide aqueous copper cyanide electroplating electrolytes containing predetermined amounts of both zinc and thiocyanate therein.

Another object of the invention is to provide an addition agent containing both zinc and thiocyanate capable of being readily dissolved in aqueous solutions to promote plating from copper cyanide electrolytes.

Other objects of the invention will in part be obvious and will in part appear hereinafter.

It has been discovered that electrodeposition of copper by means of periodic reverse current from a copper cyanide electroplating electrolyte containing both zinc and thiocyanate in predetermined amounts enables markedly improved copper electrodeposits to be obtained as compared to the same electrolyte without the addition agents or with the electrolyte containing either one of the addition agents zinc or thiocyanate alone. While ordinarily the combination of two or more addition agents in an electrolyte does not improve electrodeposition and, in fact, in some cases impairs the electrodeposition and only in rare cases improves electrodeposition, as compared to the results secured with either agent used alone, unexpected results are obtained from the combination of zinc and thiocyanate addition agents with periodic reverse current.

Specifically, outstanding copper electrodeposits have been obtained from cyanide copper electrolytes containing jointly from 0.004 to 0.57 ounce per gallon of dissolved zinc and from 0.1 to 10 ounces per gallon of thiocyanate (CNS<sup>-</sup>) in the electrolyte. The optimum proportions have been found to be from 0.05 to 0.2 ounce per gallon of zinc and from 0.5 to 2.0 ounces per gallon of thiocyanate. Tests have shown that the presence of zinc in amounts greater than 0.57 ounce per gallon is detrimental to the plating, while amounts of zinc less than 0.004 ounce per gallon produces no benefit. Thiocyanate present in an amount less than 0.1 ounce per gallon gives no benefits, while above 10 ounces per gallon its benefits decrease markedly. When a periodic reverse current is employed to electrodeposit copper from a copper cyanide electrolyte having both of these addition agents present in the effective range of proportions, smooth, hard, bright and uniform deposits of copper have been obtained over a wide range of current densities. In all cases, the quality of the copper has been superior to that produced by direct current from any known electrolyte. Many electrodeposits of copper have been secured by the practice of the present invention that have unique characteristics as will be set forth in detail hereinafter.

The electrolytes from which copper is to be electroplated may be potassium cyanide electrolytes, sodium cyanide electrolytes, mixed potassium and sodium cyanide electrolytes, and Rochelle copper cyanide electrolytes; and when the zinc and thiocyanate are introduced therein in the proportions herein set forth, the electrodeposition of copper by periodic reverse current is markedly benefited.

A copper cyanide electroplating electrolyte may be prepared with from 2 to 15 ounces per gallon of dissolved copper, an alkali metal cyanide in an amount to complex the copper in solution, that is, to produce the more soluble alkali metal-copper cyanide double salt, and in addition to provide for 0.5 to 5 ounces per gallon of

free alkali metal cyanide, from 2 to 8 ounces per gallon of alkali metal hydroxide, from 1 to 20 ounces per gallon of alkali metal carbonate, from 0.004 to 0.57 ounce per gallon of zinc and from 0.1 to 10 ounces per gallon of thiocyanate (CNS<sup>-</sup>). The pH of the cyanide solutions is usually maintained at 12 to 13 and slightly higher. The electrolyte may contain other components commonly present in cyanide copper electroplating electrolytes such, for example, as 3 to 8 ounces per gallon of Rochelle salts (potassium sodium tartrate).

The zinc may be introduced into the electrolyte as one or more of a number of zinc salts such, for example, as zinc oxide, zinc cyanide, or zinc thiocyanate; or it may be added by introducing a zinc anode into the electrolyte and passing a deplating current to dissolve the zinc in the solution. The thiocyanate may be added as an alkali metal thiocyanate such, for example, as sodium or potassium thiocyanate, or as a copper thiocyanate, or as a zinc thiocyanate salt. We have found that the following prepared compositions are most satisfactory for introducing both the zinc and thiocyanate into the electrolyte: A composition of from 0.5 to 2 parts by weight of zinc oxide, from 1 to 10 parts by weight of copper thiocyanate, and sufficient alkali metal cyanide to render the zinc oxide and copper thiocyanate readily soluble in water, the alkali metal cyanide not exceeding 20 parts by weight. The following specific composition has been used with success: 1 part zinc oxide, 2 parts copper thiocyanate and 5 parts sodium cyanide. When introduced into an electrolyte in the proportions of 1 ounce per gallon, this specific composition provides close to 0.1 ounce per gallon of zinc and 0.18 ounce per gallon of thiocyanate. There is sufficient sodium cyanide present to render the zinc oxide and copper thiocyanate readily soluble in the aqueous electrolyte.

Another composition that has been found satisfactory is prepared by combining 1 part of either zinc oxide or zinc cyanide, or a mixture of both, with from 1 to 25 parts by weight of an alkali metal thiocyanate such as sodium thiocyanate or potassium thiocyanate.

One important operating advantage derived by the use of combined zinc and thiocyanate additions in copper cyanide electrolytes is that the resulting electrolyte can be treated with activated carbon and filtered with very little loss of either zinc or thiocyanate. Metal thiocyanates are considered to be inorganic compounds. The commonly used organic addition agents, which are usually quite expensive, are removed rather completely from copper cyanide electrolytes when subjected to the same treatment. Therefore, the expense of replenishment of removed addition agent is avoided. Because of this fact, the electrolytes of the present invention can be economically treated with activated carbon at any time to remove impurities and thereby are maintainable in most efficient condition.

As disclosed in the patent to Jernstedt, No. 2,451,341, a member to be plated by periodic reverse current in the electroplating electrolytes of this invention has applied to it a plating electric current, to render the member a cathode, for plating copper from the electrolyte thereon, for a period of time of not over 40 seconds. With the electrolytes of the present invention, the plating period may be as short as 5/100 of a second. After an increment of copper has been plated on the member, then a deplating electric current is ap-

plied to the member, to render it an anode, to deplate a part of the previously plated copper, the deplating electric current being applied for a sufficient period of time and being of such a magnitude that at least 10% of the coulombs applied during the preceding plating period is applied so that a substantial part of the copper is deplated. This leaves an increment of sound, homogeneous and uniform copper on the member. Repetition of the plating and deplating electric current cycle builds up a progressively smoother and more uniform copper electrodeposit on the member. It has been found that for some purposes the deplating current may be as much as 75% of the plating current or higher with exceptionally good deposits being secured. The ratio of coulombs of plating current to deplating current may be varied in accordance with the required quality, such as brightness, smoothness or uniformity, of the deposit. The deplating current density will ordinarily be the same as the plating current density since it is most convenient in the majority of plating applications to reverse a relatively-constant, continuous direct current by means of suitable switches and timers. However, advantages have been found to accrue if the deplating current density is greater than the plating current density. The deplating current density may be double, triple or even higher than the plating current density with advantages arising. However, the deplating current density cannot be reduced to below 75% of the plating current density without loss of benefits of the periodic reverse current benefits at the preferred conditions. The following examples are illustrative of the practice of the invention:

*Example I*

An aqueous copper cyanide electrolyte of the following composition was prepared:

|                        |                                                                   |
|------------------------|-------------------------------------------------------------------|
| Copper (as a metal)    | 6 ounces per gallon.                                              |
| Potassium hydroxide    | 6 ounces per gallon.                                              |
| Free potassium cyanide | 1 ounce per gallon.                                               |
| Zinc cyanide           | Sufficient to provide 0.1 ounce per gallon of zinc.               |
| Potassium thiocyanate  | Sufficient to provide 0.5 ounce per gallon of thiocyanate (CNS-). |

The temperature of the electrolyte was 180° F. Copper was electroplated from this electrolyte using a periodic reverse current of 5 seconds plating and 1 second deplating. In the range of 13 to 105 amperes per square foot, practically mirror-bright copper was produced from the electrolyte; from 105 to 135 amperes per square foot, mirror-bright copper plate that was extremely smooth and uniform resulted; from 135 to 160 amperes per square foot, the copper electrodeposit again was nearly mirror bright.

The zinc content of the electrolyte of Example I was increased to 0.2 ounce per gallon of zinc, and the thiocyanate content was increased to 1.5 ounces per gallon. Very nearly the same results were obtained in plating over the range of 13 to 160 amperes per square foot.

*Example II*

An aqueous copper cyanide electrolyte was prepared with the following composition:

|                        | Ounces per gallon |
|------------------------|-------------------|
| Copper (as a metal)    | 8                 |
| Potassium hydroxide    | 5                 |
| Free potassium cyanide | 1/2               |

To this electrolyte there was added 1 ounce per gallon of a composition comprising 1 part by

weight of zinc oxide, 2 parts by weight of copper thiocyanate, and 5 parts by weight of sodium cyanide. A periodic reverse current having a cycle of plating for 5 seconds and deplating for 1 second was employed for plating copper from this electrolyte on members. It produced mirror-bright copper at current densities of up to 110 amperes per square foot and very bright copper plate up to and beyond 130 amperes per square foot.

The composition of Example II was employed for plating heavy deposits of copper using a periodic reverse current of 15 seconds plating and 7 seconds deplating. In this case, the work consisted of a record matrix that was rotated in the electrolyte at 60 R. P. M. with moderate agitation of the solution. The current density in both the plating and deplating cycles was 80 amperes per square foot. In 8 hours a 0.032 inch thick deposit of copper that was mirror bright and smooth was produced. Heretofore, the best plating practice required from 18 to 24 hours to plate a deposit of copper on the record matrix, and the resulting copper deposit was quite nodular and rough so that it required machining to remove beads and nodules from the edges and back side of the plate. The plated deposit produced in accordance with the present invention required no machining whatever. However, the main differences between the best previous copper deposits and that of Example II were the outstanding hardness and the superior physical characteristics of the copper deposit produced by the present invention. The copper plates produced in accordance with this Example were of a hardness of over 100 on the Rockwell F scale, whereas previously a hardness of 70 was regarded as normal. The copper plate produced in accordance with the present invention was elastic and could be bent considerably without permanent distortion, whereas the previous direct-current deposits would take a permanent set if bent to the same extent.

When the electrolyte of Example II was employed for direct-current plating, the deposits were of a light matte texture at current densities of from 20 amperes per square foot to 130 amperes per square foot and were dark matte when plated above 130 amperes per square foot and below 20 amperes per square foot. Without the zinc and thiocyanate, the same electrolyte produced deposits with direct current having a medium fogged appearance when plated at current densities of 12 amperes per square foot, and dark matte from 12 to 30 amperes per square foot, and light matte above 30 amperes per square foot.

*Example III*

An electrolyte was prepared as in Example II with an additional 0.1 ounce per gallon of zinc added as zinc oxide and 0.175 ounce per gallon of thiocyanate added as potassium thiocyanate. When plated with periodic reverse current having a cycle of 5 seconds plating and 1 second deplating, mirror-bright deposits were obtained at current densities of up to 150 amperes per square foot.

The electrolyte of Example III had added to it an additional 0.25 ounce per gallon of zinc thiocyanate. Bright deposits were obtained with periodic reverse current having cycles of 5 seconds plating and 1 second deplating at current densities of up to 150 amperes per square foot.

When a further 0.5 ounce of zinc thiocyanate was added to the electrolyte of Example III,

bright deposits were obtained up to 150 amperes per square foot.

*Example IV*

An aqueous cyanide electrolyte was prepared with:

|                     | Ounces per gallon |
|---------------------|-------------------|
| Copper              | 6                 |
| Free cyanide        | 0.75              |
| Potassium hydroxide | 5                 |
| Potassium carbonate | 5                 |

To this electrolyte was added 1 ounce per gallon of a composition composed of 1 part zinc oxide, 2 parts of copper thiocyanate and 5 parts of sodium cyanide, thereby providing 0.1 ounce per gallon of zinc and 0.18 ounce of thiocyanate. A cylinder was plated in this electrolyte by immersing one third of the periphery in the electrolyte, the cylinder being rotated at a speed of 225 revolutions per minute while being plated. The cylinder had applied to it a periodic reverse current of 15 seconds plating and 3 seconds deplating at a current density of 300 amperes per square foot of immersed area during both parts of the cycle. In two hours the entire surface of the cylinder was coated with 0.006 inch thick of copper. The plated copper was mirror bright and smooth. The surface roughness of the copper was approximately 2 micro-inches whereas the original cylinder surface had a roughness of more than 8 micro-inches (rms).

*Example V*

An aqueous cyanide electrolyte of the following composition was prepared:

|                                 | Ounces per gallon |
|---------------------------------|-------------------|
| Copper                          | 12.5              |
| NaOH                            | 7.5               |
| Free NaCN                       | 1.75              |
| Na <sub>2</sub> CO <sub>3</sub> | 3.5               |
| Zinc                            | 0.08              |
| Thiocyanate (CNS <sup>-</sup> ) | 0.15              |

This electrolyte was employed for copper plating fabricated steel members and various zinc die castings used in commercial automobiles using periodic reverse currents having the following time periods:

| Plating,<br>seconds | Deplating,<br>seconds |
|---------------------|-----------------------|
| (a) 15              | 5                     |
| (b) 15              | 3                     |
| (c) 5               | 1                     |

The current density used was varied in different tests using these time cycles of reverse current, from 20 amperes per square foot to over 60 amperes per square foot, and in all cases smooth, mirror bright, dense deposits of copper were produced.

The following cycles of periodic reverse current may be employed in practicing the invention using the electrolytes herein disclosed:

| Plating,<br>sec. | Deplating,<br>sec. |
|------------------|--------------------|
| 1                | 0.25               |
| 10               | 2                  |
| 20               | 10                 |

The electrolyte must be replenished with the addition agent particularly to provide for main-

taining the quantity of zinc, a small part of which is plated out with the copper the copper plate analyzing 99.7% copper in Example I, the balance being mainly zinc. The combination of both addition agents as salts disclosed herein may be added without the thiocyanate building up to detrimental quantities. Drag-out losses will tend to maintain the proportions of both addition agents within proper limits providing the zinc and thiocyanate are added in suitable amounts at regular intervals.

It will be appreciated that the cyanide electrolytes in the above examples are exemplary and not exhaustive. In general, it may be stated that any cyanide electrolyte from which copper may be plated by continuous direct current may be treated to add thereto both zinc and thiocyanate and used with periodic reverse current in accordance with this invention, with substantial improved plating obtained.

The electrolytes may be agitated or stirred with advantage while plating with periodic reverse current. Filtering of the electrolyte, preferably continuously, is recommended to secure electrodeposits of the optimum quality.

The preparation of the base members to be plated with periodic reverse current should be such as to produce a chemically clean surface as is conventional in order to secure the desired adherence of the metal to the base member. The preparation of the base member, therefore, may include brushing, grinding, sandblasting, shot blasting, degreasing, electrolytic cleaning and the like.

Various types and kinds of base members may be plated. Metallic bodies on which metal may be plated from conventional electrolytes may be electroplated by periodic reverse current. Carbon and graphite forms may be so electroplated. Electrotypes and electroforming base members consisting of wax or resinous patterns plated or coated with powdered graphite or precipitated silver may be electroplated as disclosed herein and the electrodeposited metal stripped therefrom. It will be found that electrotypes, molds and other electroformed members produced in accordance with the present invention will give a superior reproduction of the surface.

The copper electrodeposits produced by the use of periodic reverse current in accordance with the present invention may be plated subsequently with one or more other metals applied with similar periodic reverse current or by any other desirable process, such as by continuous direct current. In many cases, it has been found that the outstanding smoothness of the copper electrodeposits of the present invention enables the plating of subsequent metals even by continuous direct current or other conventional process to great advantage since the smoothness of the surface beneficially affects the subsequent plating. Thus, we have been able to plate an initial layer of copper with periodic reverse current and thereafter plated, nickel and chromium by direct current, and the nickel and chromium were so bright that no buffing was required. The periodic reverse current produces metal deposits that are so homogeneous and free from pores and other flaws that they possess an improved corrosion resistance for a given thickness over the same metal applied by continuous direct current.

It is intended that all the matter contained in the above description shall be deemed to be illustrative and not limiting.

We claim as our invention:

1. In the process of electroplating on a member electrodeposits of copper from an aqueous copper cyanide electroplating electrolyte, the steps comprising applying to the member the aqueous cyanide electrolyte having dissolved therein from 2 to 15 ounces per gallon of copper, between 0.004 and 0.57 ounce per gallon of zinc and thiocyanate (CNS<sup>-</sup>) in an amount of between 0.1 and 10 ounces per gallon, causing a 10 plating electric current to flow through the member while in contact with the electrolyte for a period of time of not over 40 seconds to electroplate copper on the member, then causing a deplating electric current of a sufficient magnitude to flow through the member for a period of time to deliver at least 10% of the coulombs delivered during the preceding plating period to deplate a part of the copper plated on the member, and continuing the alternate plating and deplating until a desired thickness of copper has been deposited on the member, the zinc and the thiocyanate present in the electrolyte in the given proportions resulting in the plating of a brighter and smoother electrodeposit of the copper.

2. In the process of electroplating on a member electrodeposits of copper from an aqueous copper cyanide electroplating electrolyte, the steps comprising applying to the member the aqueous cyanide electrolyte having dissolved therein from 2 to 15 ounces per gallon of copper, between 0.05 and 0.2 ounce per gallon of zinc and thiocyanate (CNS<sup>-</sup>) in an amount of between 0.5 and 2.0 ounces per gallon, causing a plating electric current to flow through the member while in contact with the electrolyte for a period of time of not over 40 seconds to electroplate copper on the member, then causing a deplating electric current of a sufficient magnitude to flow through the member for a period of time to de-

liver at least 10% of the coulombs delivered during the preceding plating period to deplate a part of the copper plated on the member, and continuing the alternate plating and deplating until a desired thickness of copper has been deposited on the member, the zinc and the thiocyanate present in the electrolyte in the given proportions resulting in the plating of a brighter and smoother electrodeposit of the copper.

3. An aqueous cyanide electroplating electrolyte composed of from 2 to 15 ounces per gallon of copper, alkali metal cyanide in an amount to complex the copper in solution and to provide from 0.5 to 5 ounces per gallon of free alkali metal cyanide, from 2 to 8 ounces per gallon of alkali metal hydroxide, from 1 to 20 ounces per gallon of alkali metal carbonate, from 0.004 to 0.57 ounce per gallon of zinc and from 0.1 to 10 ounces per gallon of thiocyanate, the zinc and thiocyanate jointly enabling smoother and brighter copper electrodeposits than either alone.

GEORGE W. JERNSTEDT.  
JAMES D. PATRICK.

25 References Cited in the file of this patent

UNITED STATES PATENTS

| Number    | Name            | Date          |
|-----------|-----------------|---------------|
| 2,146,439 | Oplinger        | Feb. 7, 1939  |
| 2,287,654 | Wernlund et al. | June 23, 1942 |
| 2,347,448 | Wernlund        | Apr. 25, 1944 |
| 2,402,185 | Schweikher      | June 18, 1946 |
| 2,451,341 | Jernstedt       | Oct. 12, 1948 |
| 2,524,912 | Jernstedt       | Oct. 10, 1950 |

30 35 OTHER REFERENCES

Ser. No. 351,241, Weiner (A. P. C.), published May 18, 1943.

40 Meyer et al., Transactions of the Electrochemical Society, vol. 73 (1938) pp. 384, 400, 401.